

## 1

3,547,626  
PLATING TARNISH-RESISTANT  
BRIGHT WHITE ALLOY  
Gaetano T. Viglione, Lexington, Mass.  
(R.D. 1, Amesbury, Mass. 01913)  
No Drawing. Filed July 2, 1968, Ser. No. 741,896  
Int. Cl. C22c 17/00  
U.S. Cl. 75—151

4 Claims

## ABSTRACT OF THE DISCLOSURE

A plating bath, process and alloy comprising cadmium, silver and nickel for tarnish-resistant bright silver applications. An alkaline cyanide water bath is employed. The alloy composition is 50 to 70% by weight of cadmium, 20 to 31% by weight of silver, balance nickel and impurities.

The present invention relates to electrolytes, electroplating processes and alloys for tarnish-resistant bright silver applications.

A purpose of the invention is to deposit a tarnish-resistant bright white silver alloy which resembles the noble metals, especially rhodium, but is much more economical.

A further purpose is to plate a tarnish-resistant bright silver alloy from an alkaline cyanide water bath containing cadmium ion, silver ion and nickel ion.

A further purpose is to employ in the alkaline cyanide water bath 0.45 to 0.55 gram per liter of cadmium ion, 0.112 to 0.138 gram per liter of silver ion and 0.675 to 0.825 gram per liter of nickel ion.

A further purpose is to plate from a preferred alkaline cyanide water bath containing 0.5 gram per liter of cadmium ion, 0.125 gram per liter of silver ion and 0.75 gram per liter of nickel ion.

A further purpose is to deposit an alloy of cadmium, silver and nickel in an attractive tarnish-resistant bright rhodium-like deposit which is effective in coverage and continuity, firmly adherent and resistant to the forces of deterioration commonly encountered by jewelry for a reasonable time.

A further purpose is to produce an alloy having by weight 50 to 70%, preferably 56 to 64% of cadmium, 20 to 31%, preferably 23 to 28% of silver and the balance nickel and impurities.

A further purpose is to produce an alloy having by weight 64% cadmium, 23% silver and the balance nickel and impurities.

A further purpose is to produce an alloy having by weight 56% cadmium, 28% silver and the balance nickel and impurities.

A further purpose is to electroplate at a temperature of 70 to 120° F.

A further purpose is to employ a current density of 5 to 60 amperes per square foot and preferably 15 to 30 amperes per square foot.

A further purpose is to employ in the cyanide plating bath an adequate quantity of an alkali such as sodium or potassium hydroxide, for example 7 to 21 grams per liter.

A further purpose is to electroplate on a base of any of the common metals suitable for jewelry and the like, for example steel, copper, brass, and bronze, applying the electroplating of the invention directly, or if desired with intermediate layers, such as copper plating or nickel plating.

Further purposes appear in the specification and in the claims.

## 2

The present invention is believed to find its best application in the decorative arts, such as the production of jewelry, trim for vehicles, decorative surfaces of appliances and machines, and for corrosion protection where appearance is important, as for example in instruments and the like.

In the prior art electrodeposited coatings including noble metals such as rhodium have been extensively developed as embodied in Keitel U.S. Patent 1,779,436, granted Oct. 28, 1930 for Process of Electrodepositing metals of the Platinum Group; Zschiegner U.S. Patent 1,779,457, granted Oct. 28, 1930, for Electrodeposition of Platinum Metals; Bart U.S. Patent 1,947,180, granted Feb. 13, 1934, for Tarnish-Resisting Silver; and Zimmermann U.S. Patent 1,981,820, granted Nov. 20, 1934, for Process of Electrodepositing Rhodium, Bath and Method of Preparing the Same.

The present invention is concerned with the production of a bright silver alloy which is much less expensive than a noble metal, but which has resistance against tarnishing in the presence of industrial atmospheres of the type encountered in cities, has adequate grain structure to provide corrosion resistance, has firm adherence to the base metal, and resistance to scuffing and abrasion of the type likely to be encountered by jewelry, trim, instrument parts, and the like. In addition the alloy of the invention is produced in a single electroplating step from a single plating bath at high speed, with a permissibly high deposition rate, and repetitively with good assurance that the same result will be obtained when all variables are controlled.

The electrodeposited layer can be applied with adequate appearance for many jewelry parts in a matter of a minute or less in order to obtain a plating layer having a thickness of the order of 0.00001 inch, or it can be applied for the purpose of electroforming in order to make a thick deposit, having a thickness for example as great as 1/4 inch or even greater.

The alloy of the invention lends itself to deposition on the common metals used in making inexpensive jewelry, trim and instrument part, such as carbon and alloy steel, copper and the copper base alloys such as brass and bronze. The coating of the invention can also be applied over prior electrodeposited layers which are employed for example for corrosion protection or to obtain a favorable color background, as copper or nickel plate on steel.

One of the great advantages of the alloy of the invention is that it has a whiteness and reflectance when polished resembling the platinum group metals, and particularly closely similar to that of rhodium plate.

The alloy of the invention resists tarnishing. For example, it has been subjected to concentrated sodium sulphide solution at 120° F. for 30 minutes without any visible impairment in the brightness of the plated surface.

Also, the alloy of the invention resists attack from alkalis in concentrations which are likely to be encountered by jewelry and trim.

The electroplating according to the invention is carried out in a cyanide water bath which of course is maintained alkaline, for example by the presence of sodium or potassium hydroxide, for instance in a concentration of 7 to 21 grams per liter.

The electrolyte has dissolved in it soluble salts providing cadmium ion, silver ion and nickel ion. In order to create such ions in the bath, the respective cyanides may be introduced or well known techniques may be used. For example cadmium oxide may be placed in the bath and dissolved by adding sodium cyanide. It will be evident of course that the conductivity of the bath can be increased if desired by adding sodium cyanide or other alkaline conducting salts.

It is very desirable to maintain a proper balance of the concentration of cadmium ion to the concentration of silver ion and the concentration of nickel ion. Very good results are obtained in an electrolyte having 0.45 to 0.55 and preferably 0.5 gram per liter of cadmium ion, 0.112 to 0.138 and preferably 0.125 gram per liter of silver ion, and 0.675 to 0.825 and preferably 0.75 gram per liter of nickel ion.

The bath temperature can vary widely but good results can be obtained in a temperature range between 70° F. and 120° F. The bath is preferably maintained at a temperature of 100° F., plus or minus 0.5° F.

The voltage employed will suitably be in the range of 2 to 12 volts direct or unidirectional current. The current density will typically vary between 5 and 50 amperes per square foot and preferably between 15 and 30 amperes per square foot. For best results an insoluble anode will be employed, such as stainless steel, platinum, titanium or carbon (graphite). The work will be the cathode, typically mounted by wire or on a rack. The ratio of anode to cathode should not exceed 0.5:1.

The alloy obtained is an alloy of cadmium, silver and nickel. In its more specific aspect it has the following composition in percentage by weight in broad and preferred ranges:

| Component                                  | Broad   | Preferred |
|--------------------------------------------|---------|-----------|
| Cadmium.....                               | 50-70   | 23-64     |
| Silver.....                                | 20-31   | 23-28     |
| Nickel and a small amount of impurity..... | Balance | Balance   |

The impurity will typically be 0.5% by weight maximum.

#### EXAMPLE 1

The following electrolyte bath was made up in water:

|                        | Grams per liter |
|------------------------|-----------------|
| Cadmium ion .....      | 0.5             |
| Silver ion .....       | 0.125           |
| Nickel ion .....       | 0.75            |
| Sodium hydroxide ..... | 15.0            |
| Sodium cyanide .....   | 7.0             |

The cadmium was added as oxide. The silver was added as cyanide. The nickel was added as cyanide.

Components suitable for jewelry were made up consisting of low carbon steel, copper and brass. Cleaning was carried on to remove grease, foreign matter and oxide as well known in the art according to 2 Metals Handbook (8th ed. 1964) 307 and following.

The bath was heated to 100° F., plus or minus 0.5° F., maintained within that temperature range and constantly stirred. An insoluble anode (stainless steel) was used, at an anode to cathode ratio of 0.5:1. The work was inserted as cathode and direct current was applied between the anode and cathode under a voltage of 1 to 1½ volts and at a current density of 15.0 amperes per square foot. The work was electroplated for 60 seconds in the above bath under the above conditions and a deposit was obtained without burnishing which was silvery white and bright. No porosity was visible and the coating was tar-

nish-resistant after immersion in concentrated sodium sulphide at 120° for 30 minutes.

Spectrographic analysis showed that the electrodeposit had the following composition by weight:

|                                              | Percent |
|----------------------------------------------|---------|
| Cadmium .....                                | 64      |
| Silver .....                                 | 23      |
| Nickel plus a small amount of impurity ..... | Balance |

#### EXAMPLE 2

The process of Example 1 was carried out except that a voltage of 3 to 4 volts was used at a current density of 30 amperes per square foot. The results were in general similar to those obtained in Example 1.

The spectrographic analysis of the electrodeposited layer in this case had the following composition by weight:

|                                              | Percent |
|----------------------------------------------|---------|
| Cadmium .....                                | 56      |
| Silver .....                                 | 28      |
| Nickel plus a small amount of impurity ..... | Balance |

The thickness of the deposits obtained in these cases were about 0.00001 inch. The deposits were subjected to scuffing and abrasion and were found to be adherent and resistant and sufficiently ductile to stand such treatment.

A wide variety of alloy compositions can be obtained by adjusting the bath efficiency (conductivity) and the current density, with or without adjustment of metal content of the bath.

No evidence has been found of porosity which could impair corrosion resistance.

It has been found that the pH range of the bath is suitably between 11.2 and 12.5.

In view of my invention and disclosure, variations and modifications to meet individual whim or particular need will doubtless become evident to others skilled in the art to obtain all or part of the benefits of my invention without copying the process and composition shown, and I, therefore, claim all such insofar as they fall within the reasonable spirit and scope of my claims.

Having thus described my invention, what I claim as new and desire to secure by Letters Patent as:

1. A tarnish-resistant bright ternary alloy essentially consisting of 50 to 70% by weight of cadmium, 20 to 31% by weight of silver, the balance being nickel and impurities.

2. An alloy of claim 1, essentially consisting of 56 to 64% by weight of cadmium, 23 to 28% by weight of silver, and the balance nickel and impurities.

3. An alloy of claim 2, essentially consisting of 64% cadmium, 23% silver and the balance nickel and impurities.

4. An alloy of claim 2, essentially consisting of 56% cadmium, 28% silver and the balance nickel and impurities.

#### References Cited

#### UNITED STATES PATENTS

2,182,380 12/1939 Hensel ..... 75—151

60 RICHARD O. DEAN, Primary Examiner